

T. J. FAY,  
PROCESS OF TEMPERING METALS,  
APPLICATION FILED JUNE 1, 1914.

1,318,367.

Patented Oct. 14, 1919.



Witnesses:

R. L. Brack.  
H. B. Mc Gill.

Inventor,

Thomas J. Fay,  
By his Attorneys, Huell & Smith.

# UNITED STATES PATENT OFFICE.

THOMAS J. FAY, OF BROOKLYN, NEW YORK, ASSIGNOR, BY MESNE ASSIGNMENTS, TO THE STANDARD PARTS COMPANY, OF CLEVELAND, OHIO, A CORPORATION OF OHIO.

## PROCESS OF TEMPERING METALS.

1,318,367.

Specification of Letters Patent. Patented Oct. 14, 1919.

Application filed June 1, 1914. Serial No. 841,982.

To all whom it may concern:

Be it known that I, THOMAS J. FAY, a citizen of the United States, residing at Brooklyn, in the county of Kings and State of New York, have invented a certain new and useful Improvement in Processes of Tempering Metals, of which the following is a full, clear, and exact description, reference being had to the accompanying drawings.

This invention relates to the tempering of metals and more particularly to a process and apparatus whereby the articles to be tempered are maintained at a uniform temperature throughout their length and without liability to burn. In carrying out my invention I make use of a bath of granular refractory material (preferably quartz sand) which, by the apparatus employed, is maintained at a uniform temperature throughout its entire extent and which temperature is sufficient to heat the articles to a sufficient degree to enable them to be tempered by subsequently subjecting them to a quenching bath in the usual manner. While capable, broadly speaking, of utilization for the heat treatment of various articles, it is particularly well adapted for the heat treatment of vehicle springs, and the embodiment herein set forth is designed with special reference to the treatment of plates of the type that enter into the construction of such springs.

In order to produce a satisfactorily and uniformly tempered product—especially in the art of spring making—it is important that the steel plates be not subjected to excessive temperatures, which will "burn" the steel; it is further important that the temperature to which the different plates are heated shall be uniform. I secure the foregoing desiderata, as well as others which will be pointed out hereinafter, in and through my process and apparatus set forth herein.

In the drawings annexed hereto and forming part hereof, Figure 1 represents a vertical, transverse sectional view through a furnace constructed in accordance with my invention and adaptable for the realization of my process; and Fig. 2 a vertical, longitudinal sectional view through the said furnace, the position of the flues on the part

of the furnace which is removed by the plane of section being indicated in broken lines.

Describing by reference characters the parts illustrated herein, 1 denotes the front, 2 the rear, 3 the side walls, and 4 the arched top of a furnace. These walls are composed of suitable refractory material. The front wall is provided with a central opening 5 into the lower part whereof there projects an injector burner nozzle 6 adapted to supply a mixture of hydrocarbon fuel (as oil) with a gaseous fluid (as steam or air, or both) into the combustion chamber 7 in the bottom of the furnace. 8 denotes an impact and distributing block of refractory material against which the burner nozzle is adapted to discharge, the block, when heated, facilitating the combustion of the fluid mixture discharged thereagainst in addition to distributing the flame in and throughout the combustion chamber.

The side and end walls are provided with ledges 9, 10 and 11 forming a seat for a refractory block 12 covering the top of the chamber 7. This block supports a large pan 13 which may be of cast iron or other suitable heating-resistant material.

Above the block 12 and between the same and the top or roof 4 is a tempering chamber 14, which communicates with the combustion chamber 7 by means of the flues 15 in the side walls 3. The number of these flues will vary with the length of the chambers 7 and 14. In the drawing, four such flues are provided in each wall 3, and the flues in one wall are staggered with respect to those in the other in order to facilitate even distribution of the gases of combustion throughout the tempering chamber 14. Outlet flues 16 serve to discharge the products of combustion from the chamber 14. The pan 13 contains a quantity of finely divided granular material, such as quartz sand, the depth of the material being sufficient to receive therewithin and entirely cover the plates 17 when placed on edge therein, the sand (or finely divided refractory material) being indicated at 18. In practice I have found quartz sand to be particularly efficient in the realization of my process as it is so mobile as to permit the steel plates to be easily embedded therein; when heated to the degree desirable for tempering, this mo-

bility is increased, and no difficulty is encountered in embedding or immersing the plates therein. Furthermore it provides a heat-storing body which remains in a solid granular and infusible condition notwithstanding the temperatures to which it is subjected.

In operation, after the furnace has been "fired" for a length of time sufficient to 10 heat the sand to the desired temperature, the plates are embedded therein with their lateral faces substantially vertical, as shown in the drawing. Owing to its finely divided and heated condition, the sand is sufficiently 15 mobile to permit the plates to be embedded therein with no material resistance to this action, although affording sufficient support to the lateral faces of the plates to assist materially in maintaining them in an upright 20 position. The plates are thus protected against the licking action of the flame (and the attendant shock upon the molecules of the steel) and the plates, through the arrangement of the sand bath relative to the 25 heating flues, may be maintained in such protected condition at a temperature which will be uniform throughout the period re-

quired for the heating of each plate and which will be uniform as to all of the plates thus treated.

It will be understood that the furnace will be provided with a thermostat, suitably located and operatively connected with the fuel supply leading to the burner, whereby the temperature in the furnace and particularly in the sand bath may be maintained at the desired degree throughout the 30 operation of the furnace.

Having thus described my invention what I claim is:—

The process of tempering plates which consists in embedding the same edgewise down in a bath of finely divided granular refractory material, and maintaining said bath at a uniform temperature throughout 45 sufficient to impart to the plates embedded therein the temperature necessary for the 40 tempering operation.

In testimony whereof, I hereunto affix my signature in the presence of two witnesses. 50

THOMAS J. FAY.

Witnesses:

J. B. HULL,

BRENNAN B. WEST.